

## UNITED STATES PATENT OFFICE

2,471,414

## CONDITIONING MINERALS FOR FILM CONCENTRATION

John Dasher, Galveston, Tex., and James E. Norman, Malvern, Ark.

No Drawing. Application January 11, 1945, Serial No. 572,441

3 Claims. (Cl. 209—9)

1

This invention relates to the concentration of minerals by flotation or other filming processes, and more particularly to a method whereby results by these processes are generally improved, and in particular are such results enhanced on difficult ores that are resistant to normal methods of separation.

In the filming process methods of minerals separation the purpose is to effect as nearly perfect separation as possible of a mineral or group of minerals from another mineral or group of minerals. Perfect separations are never obtained, so for each common separation a standard is accepted.

The primary object of the present invention is to provide a method which not only gives above the standard separations on normal ores, but also permits standard results to be obtained on difficult ores which are resistant to normal methods.

In treating normal ores each increment of collector results in an increase in the recovery of the minerals being collected, but a point is reached when the proportion of undesired minerals which are collected becomes excessive. Hence higher recoveries are not profitable by normal methods. With some mineral mixtures, especially weathered ores, or materials containing a high proportion of slime, collector additions result in no appreciable increase in recovery even when recovery of desired minerals is incomplete. Instead, undesired minerals will be collected, and hence the efficiency of the process deteriorates.

In accordance with the present invention it has been found that the deficiency just indicated may be remedied by conditioning the pulp with the collector at a temperature above normal operating temperatures. The greater the temperature, the greater the effect produced. We, therefore, prefer to use a hot pulp, namely, one above 50° C. This conditioning, however, is done on a thick pulp of a density higher than that normally used in froth flotation, or fed to agglomerating tables or other concentrating equipment.

Conditioning of the pulp as just indicated consists in agitating the hot pulp with the modifying and/or collecting reagents. The degree of agitation, similar to the degree in the conditioning temperature, is important, results being enhanced from intense agitation during the heating period. At the termination of the conditioning period the conditioned pulp is then diluted with unheated liquid such as used in normal concentration methods and is then subjected to the usual separation operations.

2

The hot conditioning of the present invention is superior to conducting the separation in a heated pulp in that it not only effects heat economy by decreasing the amount of liquid to be heated, but also it usually gives a more selective separation than is obtainable by flotation in a hot pulp.

Below are given specific examples of the effect of hot conditioning in accordance with the invention. Results are given where the only known difference in treatment is that one test was made by using a heated pulp in the conditioning step, while the other test was made with conditioning at room temperature.

15

## Example 1

A sample of flotation concentrates, containing cassiterite (tin oxide) and tungsten minerals including wolframite and scheelite, was dried and shipped for further concentration by magnetic methods. These were not successful because the scheelite was lost with the tin. This treatment is very detrimental to subsequent flotation separation. Nevertheless, samples were conditioned at room temperature and at 60° C. with 15 pounds per ton caustic soda and 2 pounds per ton oleic acid which is an example of a higher fatty acid, for twenty minutes, and floated with the addition of lime slurry to precipitate excess collector and prevent a foamy froth. The froth on the hot test was good, but the cold test gave a froth that could not be controlled well by the lime addition. The rougher froth was cleaned twice in alkaline pulp with lime added.

35

| Product  | Wt. Per Cent | Assay, Per Cent |      | Distribution, Per Cent |       |
|----------|--------------|-----------------|------|------------------------|-------|
|          |              | WO <sub>3</sub> | Sn   | WO <sub>3</sub>        | Sn    |
| Hot:     |              |                 |      |                        |       |
| W Cone.  | 33.3         | 47.0            | 13.0 | 64.4                   | 13.9  |
| Midd. 2. | 6.7          | 16.0            | 29.3 | 4.4                    | 7.0   |
| Midd. 1. | 13.3         | 15.0            | 34.5 | 8.2                    | 16.2  |
| Sn Cone. | 46.7         | 11.9            | 38.0 | 23.0                   | 62.9  |
| Cold:    | 100.0        | 24.3            | 28.2 | 100.0                  | 100.0 |
| W Cone.  | 47.4         | 34.9            | 22.0 | 64.5                   | 37.3  |
| Midd. 2. | 11.2         | 20.5            | 33.2 | 9.0                    | 13.3  |
| Midd. 1. | 13.0         | 18.0            | 33.4 | 9.1                    | 15.9  |
| Sn Cone. | 28.4         | 15.7            | 32.5 | 17.4                   | 33.5  |
|          | 100.0        | 25.6            | 27.9 | 100.0                  | 100.0 |

## Example 2

Slimes decanted from the residue of acid leaching low-grade tin concentrates contain coke, elemental sulfur, undecomposed iron sulfides and a

trace of copper sulfides. A sample of pulp was filtered and washed slightly on the filter to remove the bulk of the spent acid and iron salts. It was divided and half conditioned at 70° C., and half at room temperature, with 2 pounds per ton sodium silicate and 0.4 pound per ton of a compound pine reagent which serves as a froth toughener for ten minutes. Pulps were diluted with water at room temperature and floated. The froth was cleaned once with no further addition of reagent.

10

| Product   | Wt., Per cent | Assay, Per cent |      |      | Distribution Per cent |       |       |
|-----------|---------------|-----------------|------|------|-----------------------|-------|-------|
|           |               | Sn              | Cu   | S    | Sn                    | Cu    | S     |
| Hot:      |               |                 |      |      |                       |       |       |
| Cone      | 7.0           | 3.35            | .34  | 28.0 | 1.4                   | 31.0  | 65.0  |
| Middling  | 7.7           | 19.4            | .10  | 7.61 | 8.7                   | 10.9  | 19.5  |
| Underflow | 85.3          | 18.1            | .05  | .55  | 89.9                  | 58.1  | 15.5  |
|           | 100.0         | 17.1            | .077 | 3.02 | 100.0                 | 100.0 | 100.0 |
| Cold:     |               |                 |      |      |                       |       |       |
| Cone      | 11.5          | 6.81            | .06  | 13.2 | 4.4                   | 12.3  | 67.8  |
| Middling  | 3.1           | 22.3            | .13  | 4.45 | 10.2                  | 17.6  | 16.1  |
| Underflow | 80.4          | 18.8            | .05  | .45  | 85.4                  | 70.1  | 16.1  |
|           | 100.0         | 17.2            | .057 | 2.23 | 100.0                 | 100.0 | 100.0 |

### Example 3

Three samples of leached tin slimes were obtained from the waste acid siphoned from successive leaches of low grade tin ore concentrates. Due to differences in siphoning, the grade and proportion of slimes varied. These samples were conditioned ten minutes with 7 pounds per ton sodium silicate, the first at room temperature, the other two at 70° C. Sulfur, sulfides and coke were floated with 0.4 pound per ton of a compound pine reagent which serves as a froth toughener, and cleaned once. The non-floats were deslimed by settling and decantation so that no cassiterite grains coarser than 2 microns were lost. The settled fraction was conditioned with 2 pounds per ton oleic acid for 10 minutes, the first two tests at room temperature, and the third test at 70° C. The object of these tests was to obtain a tailing that could be rejected.

5

Both samples were diluted with unheated water, 2½ pounds per ton of sulfuric acid was added, and then they were floated. Results follow:

| Treatment                        | Product     | Wt. Per Cent | Per Cent SiO <sub>2</sub> | Dist. Per Cent |
|----------------------------------|-------------|--------------|---------------------------|----------------|
| Conditioned at Room Temperature. | Concentrate | 72.2         | 13.4                      | 71.9           |
|                                  | Tailing     | 27.8         | 13.6                      | 28.1           |
|                                  |             | 100.0        | 13.48                     | 100.0          |
| Conditioned at 70° C.            | Concentrate | 53.2         | 9.6                       | 35.5           |
|                                  | Tailing     | 46.8         | 19.8                      | 64.5           |
|                                  |             | 100.0        | 14.42                     | 100.0          |

15

### Example 5

In the flotation of hematite from quartz in an extremely slimy mixture, which contained no hematite coarse enough to be recovered on tables and no quartz coarser than 200 mesh, the following comparison was made. Two samples were conditioned in a thick pulp for 5 minutes with 5 pounds per ton oleic acid and no other reagent, one at room temperature, the other at 60° C. They were then diluted to proper flotation density and floated without the addition of any reagent.

20

| Treatment                        | Product     | Wt. Per Cent | Per Cent Fe | Dist. Per Cent |
|----------------------------------|-------------|--------------|-------------|----------------|
| Conditioned at Room Temperature. | Concentrate | 27.3         | 48.2        | 60.0           |
|                                  | Middling    | 14.5         | 11.7        | 7.8            |
|                                  | Tailing     | 58.2         | 12.7        | 32.2           |
|                                  |             | 100.0        | 21.9        | 100.0          |
| Conditioned at 60° C.            | Concentrate | 26.9         | 55.4        | 71.8           |
|                                  | Middling    | 11.9         | 15.7        | 9.0            |
|                                  | Tailing     | 61.2         | 6.5         | 19.2           |
|                                  |             | 100.0        | 20.8        | 100.0          |

40

The invention claimed is:

1. The process of concentrating a cassiterite mineral mixture which comprises, forming a thick pulp containing the minerals to be separated, elevating the temperature of the pulp to substantially 50° centigrade, agitating the heated

45

| Treatment                                  | Product     | Wt. Per cent | Percent Sn | Dist. Per cent |
|--------------------------------------------|-------------|--------------|------------|----------------|
| Cold with sodium silicate, cold with oleic | Sulfides    | 4.6          | 8.36       | 2.1            |
|                                            | Concentrate | 21.6         | 52.58      | 63.1           |
|                                            | Middling    | 9.0          | 6.84       | 3.4            |
|                                            | Tailing     | 49.6         | 5.90       | 16.2           |
|                                            | -2 Mu Slime | 15.2         | 18.00      | 16.2           |
|                                            |             | 100.0        | 18.00      | 100.0          |
| Hot with sodium silicate, cold with oleic  | Sulfides    | 7.1          | 6.25       | 2.0            |
|                                            | Concentrate | 27.4         | 55.45      | 73.9           |
|                                            | Middling    | 5.6          | 13.47      | 3.6            |
|                                            | Tailing     | 44.1         | 4.23       | 9.1            |
|                                            | -2 Mu Slime | 15.8         | 14.67      | 11.3           |
|                                            |             | 100.0        | 20.55      | 100.0          |
| Hot with sodium silicate, hot with oleic   | Sulfides    | 7.3          | 3.06       | 1.6            |
|                                            | Concentrate | 28.5         | 35.77      | 73.3           |
|                                            | Middling    | 7.6          | 4.22       | 2.3            |
|                                            | Tailing     | 35.0         | .63        | 1.6            |
|                                            | -2 Mu Slime | 20.9         | 13.64      | 21.2           |
|                                            |             | 100.0        | 13.91      | 100.0          |

### Example 4

In the flotation of a particularly refractory bauxite, normal methods gave no separation between the aluminum hydrates and the clay. Two samples were conditioned with 5 pounds per ton caustic soda, 1 pound per ton sodium silicate, and 7.5 pounds per ton oleic acid for 5 minutes, the first at room temperature, and the second at 70° C.

70 pulp in the presence of a higher fatty acid collector reagent, adding unheated liquid to the hot pulp, and thereafter selectively separating the filmed mineral from the gangue.

2. The process of concentrating a bauxite mineral mixture by filming processes comprising, applying heat to a thick pulp, subjecting the heated pulp to agitation in the presence of a higher fatty

75

acid collector reagent, adding water to the pulp, and subjecting the resultant pulp to a filming process of separation.

3. The process of concentrating a cassiterite mineral mixture by filming processes comprising treating a thick pulp of the mineral mixture including oleic acid by elevating the temperature of said pulp therein to approximately 50° centigrade, agitating the pulp while at the elevated temperature, diluting the pulp with a liquid including a precipitant for excess oleic acid, and subjecting the resultant pulp to flotation process to recover the desired minerals from the pulp.

JOHN DASHER.

JAMES E. NORMAN.

REFERENCES CITED

The following references are of record in the file of this patent:

UNITED STATES PATENTS

| Number  | Name   | Date         |
|---------|--------|--------------|
| 835,120 | Sulman | Nov. 6, 1906 |

| Number    | Name       | Date          |
|-----------|------------|---------------|
| 1,116,642 | Stevens    | Nov. 10, 1914 |
| 1,182,890 | Bradford   | May 16, 1916  |
| 1,457,680 | Whitaker   | June 5, 1923  |
| 1,459,167 | Smith      | June 19, 1923 |
| 1,951,326 | De Vaney   | Mar. 13, 1934 |
| 2,205,503 | Trotter    | June 25, 1940 |
| 2,387,081 | Herkenhoff | Oct. 16, 1945 |
| 2,410,376 | Booth      | Oct. 29, 1946 |

FOREIGN PATENTS

| Number  | Country       | Date          |
|---------|---------------|---------------|
| 460,072 | Great Britain | Jan. 10, 1937 |

OTHER REFERENCES

15 Taggart Handbook of Mineral Dressing, 1945,  
pages 1,218, 1,219, 1,299.  
Gaudin Principles of Mineral Dressing, 1939,  
pages 403, 404.